# EUROPEAN PATENT SPECIFICATION

(11) **EP 0 545 893 B1**
(45) Date of publication and mention of the grant of the patent: **30.12.1998**
(21) Application number: 93100728.0
(22) Date of filing: 25.07.1988
(51) Int. Cl.: B41M 5/00, B41M 5/40

(54) **Image-receiving sheet for thermal transfer printing**
Farbstoffempfangsschicht für thermischen Farbstoffübertragungsdruck
Feuille réceptrice d'image pour l'impression par transfert thermique

(30) Priority: 24.07.1987 JP 186095/87; 24.07.1987 JP 186096/87; 15.10.1987 JP 259968/87; 11.05.1988 JP 115065/88
(43) Date of publication of application: 09.06.1993
(62) Divisional of application: 88111947.3
(73) Proprietor: NEW OJI PAPER CO., LTD., Tokyo (JP); DAI NIPPON INSATSU KABUSHIKI KAISHA, Tokyo 162 (JP)
(72) Inventor: Kondo, Hiromasa, Ikoma-shi, Nara (JP); Okumura, Yoshitaka, Ukyo-ku, Kyoto-shi, Kyoto (JP); Fukui, Terunobu, Nishinomiya-shi, Hyogo (JP); Egashira, Noritaka, Tokyo 165 (JP); Iwata, Tamami, Arakawa-ku, Tokyo (JP); Satake, Naoto, Shinjuku-ku, Tokyo (JP)
(74) Representative: Kraus, Walter, Dr.

(56) References cited:
- PATENT ABSTRACTS OF JAPAN vol. 11, no. 166 (M-593)(2613) 28 May 1987
- PATENT ABSTRACTS OF JAPAN vol. 11, no. 16 (M-554)(2463) 16 January 1987
- PATENT ABSTRACTS OF JAPAN vol. 6, no. 210 (M-166)(1088) 22 October 1982
- PATENT ABSTRACTS OF JAPAN vol. 10, no. 342 (M-536)(2398) 19 November 1986

## Description

### BACKGROUND OF THE INVENTION

### Field of the Invention

The present invention relates to an improvement in image-receiving sheets for thermal transfer printing which are adapted for printing images thereon by transfer of a sublimable dye of a thermal transfer sheet by application of heat from a thermal head in accordance with image signals. More particularly, the present invention relates to an improved image-receiving sheet with a two-layered intermediate layer for thermal transfer printing.

### Description of the Prior Art

Thermal printing systems in which printed images are obtained upon reception of input signals are made up of a relatively simple apparatus and are inexpensive and low in noises, so that they have increasing utility in various fields such as facsimiles, terminal printers for electronic computers, printers for measuring instruments, video printers, and the like.

A recording medium generally used in these thermal printing systems is a so-called color-developing, heat-sensitive recording paper having a recording layer which undergoes a physical or chemical change by application of heat to form a color. However, the recording paper of the color developing type has disadvantages in that it is liable to undesirably develop the color during the process of fabrication or during storage. In addition, the image printed on the paper is poor in storage stability and is apt to fade on contact with organic solvents or chemicals.

To avoid this, there has been proposed a thermal transfer printing system in which a recording medium utilizing a dye or colorant is used instead of the color-developing thermosensitive recording paper.

In this thermal transfer printing system, a colorant or colored dye is caused to melt, evaporate or sublimate by application of heat and transferred on a recording paper, thereby forming a record image by adhesion, adsorption or reception of the dye on the recording paper. For instance, there has been proposed a mechanism as is shown in Fig. 2. In the mechanism, a thermal transfer sheet 201 having a dye layer on a substrate and a thermal transfer image-receiving sheet 203 set on a platen roller 202 are superposed and heated from the non-faced side of the thermal transfer sheet 201 by a heating means 204 such as a thermal head. The thermal head 204 is controlled with electric signals corresponding to image information. As a result, the dye of the thermal transfer sheet is transferred on an image-receiving layer.

For full color printing, a thermal transfer sheet used is a sheet which has been coated or printed, as shown in Fig. 3, a start mark 301 and dyes including yellow 302, magenta 303 and cyan 304, and also including a black dye, if necessary. This sheet is superposed on a thermal transfer image-receiving sheet and the yellow, magenta and cyan dyes are successively heated according to the respective color-separated image signals to make an image in which the three colors are superposed. Thus, a natural color, photographic image is formed.

A known thermal transfer image-receiving sheet used in this type of printing system is one which has an image-receiving layer obtained by coating onto a paper substrate such as high-quality paper a coating of a dispersion of finely powdered silica or calcium carbonate in a binder such as a thermoplastic polyester resin.

However, when the image-receiving layer is formed on the substrate, such as wood free paper, whose smoothness is low, it is difficult to obtain a satisfactory printed image. Especially, where an image with a degree of gradation is transferred, missing transfer portions are liable to occur at half-tone to low-tone portions. Although images such as of symbols, letters and figures are substantially solid and thus the missing transfer portions are not conspicuous, missing transfer portions on photographs or colored solid images will undesirably tend to become marked and produce vital deficiencies. Accordingly, there is a strong demand for eliminating such deficiencies.

In reply to said demand, various improvements have been proposed including, for example, (1) a method proposed in Japanese Laid-open Patent Application No. 61-172795 in which an intermediate layer is formed beneath an image-receiving layer to improve a smoothness on the surface of the image-receiving layer, and (2) a method proposed in U.S. Patent No. 4,720,480 in which an intermediate layer made primarily of a flexible resin is formed.

However, these improvements are still accompanied with other problems and thus, satisfactory results cannot always be obtained. For instance, the method (1) has a problem that the productivity lowers because it comprises the step in which the intermediate layer which has been kept as softened or plastic is brought into close contact with mirror-like finished chromium plated metal drum for heating and drying. The method (2) involves the problem that a soft resin such as MBR, polyurethane, polybutadiene, SBR or the like, which has been formulated so as to improve the adhesiveness, is liable to block when wound up after coating and drying. Additionally, the resin dissolves in an organic solvent of the coating solution forming an image-receiving layer, so that the image-receiving layer cannot be formed uniformly, thus causing a lowering of an optical density of the printed image.

### SUMMARY OF THE INVENTION

An object of the invention is to provide an improved image-receiving sheet with a two-layered intermediate layer for thermal transfer printing which is free from the foregoing problems which are found on the known image-receiving sheet and which enables one to form beautiful printing images of high optical density without involving the known problem relating to a transfer missing portion.

Another object of the invention is to provide an improved image-receiving sheet with a two-layered intermediate layer which is capable of forming images of high quality having good gradation and which is free from the known problem relating to a missing transfer portion even upon using as a base sheet various paper sheets made primarily of pulp fibers.

The present inventors have made intensive studies in order to achieve the above objects and, as a result, found that when a base sheet is first formed with an intermediate layer made primarily of a resin insoluble in organic solvents and then with an image-receiving layer made chiefly of a resin soluble in organic solvents, the smoothness and the anti-blocking properties are significantly improved. And this results in making printed images beautiful without causing any missing transfer portion and making the printed images to have an excellent optical density.

The present invention has been accomplished based on the above findings.

### BRIEF DESCRIPTION OF THE DRAWINGS

Fig. 1 is a schematic sectional view of an image-receiving sheet for thermal transfer printing according to the present invention, in which 101 indicates a base sheet or substrate, 102 indicates an intermediate layer having a two-layered structure comprising a lower layer and an upper layer, and 103 indicates an image-receiving layer;
Fig. 2 is a schematic view showing a printing system of the thermal transfer type, in which indicated by 201 is a thermal transfer sheet, by 202 is a platen roller, by 203 is a sheet of receiving an image by thermal transfer, and by 204 is a thermal printing head.
Fig. 3 is a schematic view of a full-color thermal transfer sheet, in which indicated by 301 is a start mark, by 302 is a yellow color, by 303 is a magenta color, and by 304 is a cyan color.

The present invention relates to an image-receiving sheet for thermal transfer printing which comprises (a) an intermediate layer and (b) an image-receiving layer formed on a substrate in this order, characterised in that said intermediate layer (a) comprises (a-i) a lower layer and (a-ii) an upper layer formed on said lower layer (a-i), said image-receiving layer (b) being comprised primarily of a resin soluble in an organic solvent,
said lower layer (a-i) being comprised primarily of a resin insoluble in an organic solvent,
said resin being formed from a polymer latex satisfying the following requirements (1) and (2):

| | | |
|---|---|---|
| (1) | compositional constituents: | |
| | aliphatic conjugated diolefinic monomer | 20-70 wt.-% |
| | unsaturated acid monomer | 0.5-15 wt.-% |
| | other olefinic monomer | 15-79.5 wt.-% |
| (2) | gel content: | 85-100 wt.-% |

and containing hollow particles in an amount of not less than 50 wt.-% of the total solids in solid lower layer (a-i), the hollow particles having a size of 0.1-200 µm and being soluble in organic solvents, said upper layer (a-ii) being comprised of an organic-solvent resistant resin.

Fig. 1 is a schematic sectional view showing an image-receiving sheet for thermal transfer printing according to the invention. In the figure, 101 denotes a substrate, 102 denotes the above-mentioned intermediate layer, and 103 denotes an image-receiving layer.

These elements of the image-receiving sheet according to the invention will be below described in more detail.

### Intermediate Layer 102

The characteristic properties of the intermediate layer which is one of prominent features of the present invention are described in detail.

The main constituent layer of the intermediate layer of the image-receiving sheet according to the present invention contains as its primary component resins which are insoluble in organic solvents.

It has been found that when a copolymer latex having a specific type of monomer composition and a certain gel content (content of toluene-insoluble component) is used as the organic solvent-insoluble resin, the organic solvent resistance and the blocking properties of the intermediate layer are effectively improved without impeding the smoothness of the image-receiving layer. This results in efficient production of an image-receiving sheet capable of yielding printing images which are free from missing transfer portions, high in optical density and beautiful.

The monomer composition and gel content of the copolyer latex are shown below.

| Monomer Composition: | |
|---|---|
| (A) Aliphatic conjugated diolefinic monomer wt% | 20 - 70 |
| (B) Unsaturated acid monomer | 0.5 - 15 wt% |
| (C) Olefinic monomer other than said aliphatic conjugated diolefinic monomer | 15 - 79.5 wt% |
| Gel Content: | 85 - 100 wt% |

The aliphatic conjugated diolefinic monomer (A) is generally selected from those having from 4 to 10 carbon atoms. Specific examples include 1,3-butadiene, 2-methyl-1,3-butadiene, 2,3-dimethyl-1,3-butadiene, halogen-substituted butadienes, substituted linear conjugated pentadienes, linear or branched conjugated hexadienes, and the like. The aliphatic conjugated diolefinic monomer should be contained in an amount of from 20 to 70 wt% of the copolymer latex. When the content is less than 20 wt%, the resultant resin becomes hard and brittle and exhibits poor film forming properties and adhesion strength. Over 70 wt%, the resultant resin becomes too soft even when the gel content is over 85 wt%, tending to cause sticking on rolls during the course of coating or blocking.

The unsaturated acid monomer (B) includes, for example, acrylic acid, methacrylic acid, maleic acid, fumaric acid, itaconic acid, dicarboxylic acid anhydrides, dicarboxylic acid monoalkyl esters, and the like. The unsaturated acid monomer is contained in an amount of from 0.5 to 15 wt% of the copolymer latex. If the content is less than 0.5 wt%, the mechanical stability of the copolymer latex lowers, whereas over 15 wt%, the latex tends to undesirably become too viscous.

The olefinic monomer (C) other than the aliphatic conjugated diolefinic monomer (A) and the unsaturated acid monomer (B) includes, for example, aromatic vinyl monomers such as styrene, alpha-methylstyrene, dimethylstyrene vinyl toluene and the like, acrylates monomers such as methyl acrylate, ethyl acrylate, butyl acrylate, 2-ethylhexyl acrylate, lauryl acrylate, 2-hydroxyethyl acrylate, 2-hydroxypropyl acrylate and the like, methacrylate monomers such as methyl methacrylate, ethyl methacrylate, 2-hydroxyethyl methacrylate, 2-hydroxypropyl methacrylate and the like, unsaturated nitrile monomers such as acrylonitrile, methacrylonitrile and the like, and acrylamide, N-methylolacrylamide, glycidyl acrylate, glycidyl methacrylate and the like.

The gel content of the copolymer latex, which is one of important features of the invention, should be controlled in a range of from 85 to 100 wt%. Although the gel content may be influenced depending upon the monomer composition, the yield of emulsion polymerization, the polymerization temperature and the like, it should be controlled over 85 wt% by controlling an amount of a chain transfer agent such as carbon tetrachloride, dodecyl mercaptan, octyl mercaptan or the like or by appropriately using a crosslinking agent such as methylenebisacrylamide, divinylbenzene, diallyl phthalate or the like. When the gel content is less than 85 wt%, there may be the fear that blocking will occur, making it impossible to wind up a final product after coating.

It will be noted that the gel content used herein is a value determined according to the following procedure.

A latex is allowed to stand on a glass plate at room temperature (in a air-dried condition) over 24 hours, after which it is dried in vacuum for 2 to 3 hours to obtain an about 1 mm thick latex film. About 0.5 g of the thus obtained film is accurately weighed and immersed in 50 ml of toluene at room temperature for 24 hours. Subsequently, the toluene solution is passed through a 200 mesh stainless steel screen to collect an insoluble matter, followed by drying it at 135°C for 3 hours and measuring the weight. Then, the ratio (wt%) to the weight prior to the immersion in the toluene solution is calculated as the gel content.

In the practice of the present invention, the above specific type of copolymer latex should preferably be contained in the main constituent layer of the intermediate layer in an amount of not less than 60 wt%, more preferably not less than 70 wt%, of the total solid of the main constituent layer of the intermediate layer in order to obtain a desired high optical density for images as printed.

The main constituent layer of the intermediate layer may further contain various additives including pigments such as silica, alumina, clay, calcium carbonate and plastic pigments, lubricants, fluorescent dyes, and other adhesives in amounts not impeding the effects of a resin insoluble in organic solvents.

When large amounts of fine particles of inorganic pigments are added to the main constituent of the intermediate layer, the heat insulating properties and cushioning properties lower, causing the optical density to lower with an increasing number of missing transfer portions.
It has been found that when hollow particles are contained in the resin, the heat-insulating properties of the main constituent layer of the intermediate layer can be remarkably improved together with an attendant remarkable improvement in the optical density for images as printed.

The hollow particles useful for this purpose are, for example, those described below.

### (1) Thermally expandable plastic materials

Hollow particles with capsule walls made of thermoplastic materials such as vinylidene chloride-acrylonitrile copolymers and a volatile expanding agent, such as propane, n-butane, iso-butane or the like, in the inside of individual particles.

Commercially available products: Matsumoto Microsphere F-30™, produced by Matsumoto Yushi-Seiyaku Co., Ltd.; and

Expancel 551, 642™, produced by KemaNobel Company

### (2) Hollow polymers of a microcapsular form

Hard resins such as acryl-styrene copolymers are used as a shell in which water is contained and is flown away upon drying to form hollow polymer particles.

Commercially available product: Ropaque OP-84J™ (acryl-styrene copolymer), produced by Rohm & Haas Japan Kabushiki Kaisha.

The above hollow particles have a size of 0.1 to 200 micrometers. Preferably, those hollow particles having a size of from 0.1 to 20 micrometers are used.

When the size is less than 0.1 micrometer, satisfactory heat-insulating effects cannot be expected. Over 20 micrometers, the smoothness of the image-receiving layer lowers. In this connection, however, the hollow particles obtained by thermal expansion of thermally expandable plastic materials have the cushioninig action and are flexible, so that they are usable when the size is not larger than 100 micrometers.

The above-mentioned hollow particles are all soluble in organic solvents such as methyl ethyl ketone and should be used after dispersion in an organic solvent-resistant resin used as an binder.

The hollow particles are used in an amount of not less than 50 wt% of the total solids in the main constituent layer of the intermediate layer.

As above described, the intermediate layer of the image-receiving sheet according to the present invention has a two-layered structure comprising the main constituent layer and the protective layer. The protective layer is disposed on the main constituent layer comprised of the hollow particles. The protective layer serves not only to smooth the surface of the main constituent layer comprised of the hollow particles but also to provide the resulting image-receiving sheet with a desirable flexibility.

The protective layer is formed of an organic solvent-resistant resin. Specific examples of the organic solvent-resistant resin by which the protective layer is constituted are copolymer latices having specific monomer composition and gel content. Aside from the latices, resins having good film-forming properties and capable of inhibiting organic solvents from infiltrating may be used including, for example, hydrophilic polymers such as polyvinyl alcohol, casein, starch and the like, acrylic esters, ethylene-vinyl acetate copolymers, carboxyl group-containing polyethylene, and the like. Of these, the copolymer latices and the hydrophilic polymers including polyvinyl alcohol, casein, starch and the like are preferred because of good synergistic effects with the hollow particles contained in the main constituent layer.

The thickness of the main constituent layer of the intermediate layer is generally in the range of from 10 to 50 micrometers, preferably from 15 to 30 micrometers. When the hollow particles made of a thermally expandable plastic material are used, dry coating of the main constituent layer of the intermediate layer is in the range of from 1 to 10 g/m², and preferably, from 2 to 6 g/m². For non-thermally expandable hollow particles, the thickness is in the range of from 5 to 50 micrometers, preferably from 10 to 30 micrometers.

The main constituent layer of the intermediate layer may further comprise microcapsules which contain a core substance having the plasticizing action on an image-receiving layer made primarily of a resin soluble in organic solvent, e.g. esters such as phosphoric esters, (tere)phthalic esters, adipic esters and the like, polyesters in the form of oligomers of dibasic acids and glycols or glycerine, epoxy fatty acid esters, and the like. The thermal transfer image-receiving sheet obtained in this case is improved in the receptivity of sublimable dyes without involving any missing transfer portion and has a high optical density for images as printed. The wall of the capsule used above should permit thermal transmission of the core substance through the capsule wall when heated at the time of printing. For this purpose, the capsule wall is desired to be made of polyurethane or polyurea.

### Substrate 101

As the substrate 101, there may be used, for example, a synthetic paper, a wood free paper, a No.1 grade coated paper, a coated paper, a cast coated paper, polymer films, and composite sheets of these papers and films.

There are known a variety of paper sheets chiefly comprised of pulp fibers. It is commonly recognized that such paper sheet is considerably inferior to a synthetic film with respect to occurrence of missing transfer portions and the optical density for images as printed when employed as the substrate for an image-receiving sheet for thermal transfer printing and because of this, such paper sheet is not always considered to be usable as the substrate. However, in the present invention, there may be also used such paper sheet chiefly comprised of pulp fibers as the substrate 101. That is, even in the case where such paper sheet is used as the substrate 101, the image-receiving sheet to be prepared by forming a specific intermediate layer and a particular image-receiving layer thereon according to the present invention becomes to effectively attain the objects of the present invention.

Now, as a result of intensive studies by the present inventors on a paper sheet to be used as the substrate 101, it has been found that for formation of an intermediate layer having good cushioning and heat-insulating properties and high smoothness, not only the manner of formation of the intermediate layer, but also surface physical properties of the paper sheet substrate or support are very important factors. It has also been found that when the paper sheet substrate is appropriately defined with respect to the surface physical properties, an intermediate layer having desired characteristics can be very efficiently obtained.

More particularly, when the physical properties of the paper sheet substrate on the surface contacting an intermediate layer meet the following requirements, the resultant intermediate layer are imparted with very good characteristics. This results in formation of an image-receiving sheet for thermal transfer printing which can exhibit a high degree of gradation and is substantially free from the known problems relating to occurrence of missing transfer portions when printed.

### |Requirements for Surface Physical Properties of Paper Sheet|

(1) Smoothness not less than 6% when measured by means of a specular reflection smoothness tester under a pressure of 20 kg/cm².
(2) Water absorption: a 5 second value of 1 to 30 g/m² when determined according to Test Method for Water Absorption of Paper and Paperboard prescribed in JIS P-8140 (Cobb's method).

In general, the smoothness of paper sheet is measured by means of a measuring instrument such as a specular reflection smoothness tester, a Bekk smoothness tester, a Parker Print Surf or the like. According to our detailed studies, the measurement with an air leakage-type Bekk smoothness tester or Parker Print-Surf (H.E. Messmer Ltd.) is greatly influenced by air permeability of the substrate sheet. It has been found difficult to establish a correct interrelation between a measurement and an actual smoothness for various substrate sheets whose properties greatly differ from one another. Especially, when intimate contact with a thermal head or a thermal transfer sheet is an important factor as with an image-receiving sheet for thermal transfer printing, the measurement of smoothness under the conditions where a sample is pressed against a glass surface at a given pressure as in the case of the specular reflection smoothness tester has been found to be most appropriate in view of the interrelation.

Thus, the smoothness of a paper substrate sheet used in the practice of the present invention should be determined using a specular reflection smoothness tester. When a paper substrate sheet having not less than 6%, preferably not less than 7%, when measured at a pressure of 20 kg/cm² (a greater value leading to a better smoothness), is used, an intermediate layer having desired characteristics can be very efficiently formed.

It takes only several seconds after application of a coating for the main constituent layer of the intermediate layer onto a substrate till drying the coating. If, however, a degree of sizing of the paper substrate sheet is too low, the coating solution for the intermediate layer infiltrates into the sheet during the coating, making it difficult to obtain a smooth intermediate layer. Accordingly, it is necessary that the substrate sheet have a suitable degree of sizing on the surface which contacts with the intermediate layer. This is the reason why a paper substrate sheet having a 5 second value of from 1 to 30 g/m², preferably from 3 to 20 g/m², when determined by the aforementioned Test Method for Water Absorption of Paper and Paperboard is selectively used.

When the water absorption is smaller than 1 g/m², the wetting between the paper substrate sheet and the coating solution for the intermediate layer becomes poor. Thus, difficulties will be involved in that the aqueous coating solution is repelled from the substrate or the adhesiveness of the resultant layer lowers. Over 30 g/m², the infiltration of the coating solution into the paper substrate sheet becomes excessive, disenabling one to obtain a smooth intermediate layer.

The paper-base substrates are not critical with respect to the type provided that the above requirements for the surface are satisfied. Examples of the paper-base substrate includes gloss, dull and mat-type coated papers such as No.1 grade coated papers, coated papers, lightweight coated papers, finely coated papers, cast coated papers and the like, and non-coated papers such as wood free papers, medium papers, super calendered papers and the like.

### Image-receiving Layer 103

As above described, the image-receiving layer of the image-receiving sheet for thermal transfer printing according to the invention is formed primarily of resins soluble in organic solvents. Examples of the organic solvent-soluble resins are those below mentioned.
(a) Resins having ester bonds: polyester resins, polyacrylate resins, polycarbonate resins, polyvinyl acetate resins, styrene-acrylate resins, vinyltoluenecarboxylate resins and the like.
(b) Resins having urethane bonds: polyurethane resins and the like.
(c) Resins having amide bonds: polyamide resins (nylons) and the like.
(d) Resins having urea bonds: urea resins and the like.
(e) Vinyl chloride-(meth)acrylic ester copolymers
   The (meth)acylic acid monomers include: acrylic acid; acrylic acid salts such as calcium acrylate, zinc acrylate, magnesium acrylate, aluminium acrylate and the like; acrylates such as methyl acrylate, ethyl acrylate, butyl acrylate, 2-ethylhexyl acrylate, 2-ethoxyethyl acrylate, 2-hydroxyethyl acrylate, n-stearyl acrylate, tetrahydrofurfuryl acrylate, trimethylolpropane triacrylate and the like; methacrylic acid; and methacrylates such as methyl methacrylate, ethyl methacrylate, t-butyl methacrylate, tridecyl methacrylate, cyclohexyl methacrylate, triethylene glycol dimethacrylate, 1,3-butylene dimethacrylate, trimethylolpropane methacrylate and the like.
   The ratio of vinyl chloride and the (meth)acrylic acid monomer for the copolymerization is preferably vinyl chloride/acrylic acid monomer = 50 to 90%/50 to 10%. The molecular weight is generally in the range of from 5000 to 40000, preferably from 10000 to 30000.
   Aside from the above copolymers, copolymers of monomers, such as acrylonitrile, vinylpyrrolidone, N-substituted maleimides, maleic acid and the like with vinyl chloride and a (meth)acrylic acid monomer are preferably used. In this case, the ratio of the other monomers is preferably from 0.1 to 30%.
   As a matter of course, the copolymers may be used by blending with other resins.
(f) Other resins having bonds of high polarity: polycaprolactone resins, styrene/maleic acid resins, polyvinyl chloride resin, polyacrylonitrile resin and the like.

These resins have good receptivity of sublimable dyes and good storage properties and are thus favorably used in the practice of the invention. Of these resins, polyester resins and vinylchloride-(meth)acrylic ester copolymers are preferred because of their good transferability in dye stuffs and of their light fastness of transferred dye stuffs.

Apart from these resins, various additives may be added to the image-receiving layer, if necessary. Examples of such additives include mineral pigments such as, for example, titanium dioxide, zinc oxide, aluminium hydroxide, calcium carbonate, finely powdered silica and the like and organic white pigments such as plastic pigments in order to improve whiteness and thermal fusion properties, modified silicon resins, solid waxes, polyethylene waxes, amide waxes, calcium silicate, and the like. Moreover, for the purpose of stabilizing images printed, UV absorbers and light stabilizers may be added in amounts not impeding the effects of the invention.

The image-receiving layer may be formed by applying a coating composition for the image-receiving layer onto the surface of the protective layer of the intermediate layer, which has been previously formed on a substrate, in a dry thickness of from 1 to 15 micrometers, preferably from 2 to 10 micrometers by any known coating apparatus such as, for example, a bar coater, a gravure coater or the like, and drying the coating composition applied.

### PREFERRED EMBODIMENTS OF THE INVENTION

The present invention will be described in more detail by way of examples and comparative examples, which should not be construed as limiting the ivention.

### EXAMPLE 1

### 1. An image-receiving sheet with a two-layered intermediate layer for thermal transfer printing was prepared in the following manner.

### Preparation of base paper sheet

A paper stock comprised of 30 parts of bleached NKP and 70 parts of bleached LKP to which 0.4 parts of a rosin size, 10 parts of talc and 2.3 parts of aluminium sulfate were added was prepared and subjected to paper making by means of a Fourdrinier paper machine at a rate of 600 m/minute in such a way that a dry weight was 101 g/m², followed by coating a oxidized starch solution having a concentration of 6% by the use of a size press in an amount of 50 ml/m², drying and winding-up. The resultant base paper sheet was subjected to supercalendering under the following conditions.

| Supercalendering conditions: | |
|---|---|
| linear pressure | 200 kg/cm |
| surface temperature of chrominum-plated metal roll | 25°C |
| running speed of paper | 250 m/minute |
| number of nips for running paper | 4 |

After the supercalendering treatment, the base paper sheet was found to have a Cobb water absorption (5 second value) of 10.4 g/m² and a smoothness of 13% as determined by the specular reflection smoothness tester at a pressure of 20 kg/cm².

### Preparation of coated paper sheet

### (a) Preparation of a coating composition:

60 parts of ground calcium carbonate (trademark name: Sofuton 1800, produced by Bihoku Funka Kogyo Kabushiki Kaisha), precipitated calcium carbonate (trademark name: Brilliant S-15, produced by Shiraishi Calcium Kaisha, Ltd.), and 0.2 parts of sodium polyacrylate were dispersed in water by means of Coweles Dissolver (produced by Morehouse Industries, Inc.) to obtain a pigment slurry having a solid content of 55%. To the slurry were added 3 parts (as solid) of oxidized starch and 12 parts (as solid) of a modified styrene-butadiene copolymer latex (trademark name: JSR-0696, produced by Japan Synthetic Rubber Co., Ltd.), followed by further addition of water to obtain a coating composition having a solid content of 50%.

### (b) Preparation of coated paper

The coating composition thus obtained was applied onto the surface of the base paper sheet obtained in the above in an amount to provide a thickness of 25 micrometers when dried, followed by drying, to thereby obtain a coated paper sheet. The resultant coated paper sheet was subjected to supercalendering under the following conditions.

| Supercalendering conditions: | |
|---|---|
| linear pressure | 60 kg/cm |
| surface temperature of a chrominum-plated metal roll | 25°C |
| running paper speed | 5 m/minute |
| number of nips for running paper | 2 |

The coated paper sheet obtained after the supercalendering treatment was found to have a Cobb water absorption (5 second value) of 12.3 g/m² and a smoothness (under a pressure of 20 kg/cm²) of 16% when determined by a specular reflection smoothness tester.

### Formation of two-layered intermediate layer

A two-layered intermediate layer was formed in the following manner on the surface of the coated paper sheet obtained in the above.

### (a) Formation of a lower layer as the main constituent layer of the intermediate layer:

70 parts of thermally expandable hollow particles (trademark name: Matsumoto Microsphere F-30, produced by Matsumoto Yushi-Seiyaku Co., Ltd.) whose shell walls have a softening temperature of from 80 to 85°C and 30 parts of a modified styrene-butadiene latex (trademark name: JSR-0696, produced by Japan Synthetic Rubber Co., Ltd.) were agitated with a mixer, to which water was added so as to obtain a 45% coating composition.

The resultant coating composition was applied onto the surface of the coated paper sheet obtained in the above, by means of a wire bar in an amount of 3.5 g/m² on a dry weight basis, followed by drying at 120°C for 1 minute. After the drying, the thermally expandable hollow particles were individually expanded to 30 to 70 times larger, whereby the lower layer was formed.

### (b) Formation of an upper layer as the protective layer of the intermediate layer:

A coating composition comprising polyvinyl alcohol (trademark name: PVA-110, produced by Kuraray Co., Ltd.) was applied onto the surface of the lower layer formed in the above by means of a wire bar in an amount of 3.5 g/m² on a dry weight basis, followed by drying, whereby the upper layer was formed.

Thus, an intermediate layer comprising the lower layer as the main constituent layer and the upper layer as the protective layer was formed on the surface of the coated paper sheet.

### Formation of image-receiving layer

### (a) Preparation of a coating composition:

100 parts of a polyester resin (trademark name: Vylon 200, produced by Toyobo Co., Ltd.), 0.5 parts of an amino-modified silicon (trademark name: KF-393, produced by The Shin-Etsu Chemical Co., Ltd.), and 0.5 parts of an epoxy-modified silicon (trademark name: X-22-343, produced by Shin-Etsu Chem. Co., Ltd.) were added to methyl ethyl ketone/toluene (ratio by weight of 1:1) while agitating with a mixer, to thereby obtain a coating composition for the image-receiving layer having a solid content of 15%.

### (b) Formation of the image-receiving layer

The coating composition obtained in the above was applied onto the surface of the upper layer of the intermediate layer in an amount to provide a thickness of 7 micrometers when dried by means of a wire bar, followed by drying. The resultant was subjected to supercalendering under the following conditions, to thereby form an image-receiving layer on the surface of the upper layer of the intermediate layer.

| Supercalendering conditions: | |
|---|---|
| linear pressure | 90 kg/cm |
| surface temperature of a chrominum-plated metal roll | 70°C |
| running paper speed | 5 m/minute |
| number of nips for running paper | 2 |

Thus, there was obtained an image-receiving sheet for thermal transfer printing.

### 2. A thermal transfer sheet was prepared in the following manner.

### (a) Preparation of an ink composition for the formation of a thermal transfer layer:

40 parts of a sublimable disperse dye (trademark name: Kayaset Blue 714, produced by Nippon Kayaku Co., Ltd.) and 60 parts by weight of polyvinyl butyral were added to methyl ethyl ketone/toluene (ratio by weight of 1:1) while agitating with a mixer to obtain an ink composition having a solid content of 10%.

### (b) Formation of a thermal transfer layer:

The ink composition obtained in the above was applied onto a 4.5 micrometer thick PET film, whose back side had been subjected to heat-resisting treatment, in an amount of 1 g/m² on a dry weight basis by means of a wire bar, followed by drying.

Thus, there was obtained a thermal transfer sheet.

### Evaluation of the image-receiving sheet for thermal transfer printing

The thermal transfer sheet obtained in the above was superposed on the image-receiving sheet for thermal transfer printing obtained in the above, followed by printing under conditions of an output power of 1 W/dot, a pulse width of 0.3 to 4.5 msec., and a dot density of 3 dots/mm for evaluation. The evaluated results are shown in Table 1.

### EXAMPLE 2

### 1. An image-receiving sheet with a two-layered intermediate layer for thermal transfer printing was prepared in the following manner.

### Preparation of base paper sheet

A paper stock comprised of 30 parts of bleached NKP and 70 parts of bleached LKP to which 0.4 parts of a rosin size, 10 parts of talc and 2.3 parts of aluminium sulfate were added was prepared and subjected to paper making by means of a Fourdrinier paper machine at a rate of 600 m/minute in such a way that a dry weight was 101 g/m², followed by coating a oxidized starch solution having a concentration of 6% by the use of a size press in an amount of 50 ml/m², drying and winding-up. The resultant base paper sheet was subjected to supercalendering under the following conditions.

| Supercalendering conditions: | |
|---|---|
| linear pressure | 200 kg/cm |
| surface temperature of chrominum-plated metal roll | 25°C |
| running speed of paper | 250 m/minute |
| number of nips for running paper | 4 |

After the supercalendering treatment, the base paper sheet was found to have a Cobb water absorption (5 second value) of 10.4 g/m² and a smoothness of 13% as determined by the specular reflection smoothness tester at a pressure of 20 kg/cm².

### Formation of two-layered intermediate layer

A two-layered intermediate layer was formed in the following manner on the surface of the base paper sheet obtained in the above.

### (a) Formation of a lower layer as the main constituent layer of the intermediate layer:

80 parts of hollow particles of Ropaque OP-84J (trademark name, produced by Rohm & Haars Japan Kabushiki Kaisha) and 20 parts of a modified styrene-butadiene copolymer latex (trademark name: JSR-0696, produced by Japan Synthetic Rubber Co., Ltd.) were agitated with a mixer, followed by addition of water to obtain a 40% coating composition.

The resultant coating composition was applied onto the surface of the base paper sheet obtained in the above by means of a wire bar in an amount to provide a thickness of 20 micrometers when dried, followed by drying, whereby the lower layer was formed on the surface of the base paper sheet.

### (b) Formation of an upper layer as the protective layer of the intermediate layer:

A coating composition comprising polyvinyl alcohol (trademark name: PVA-110, produced by Kuraray Co., Ltd.) was applied onto the surface of the lower layer by means of a wire bar in an amount of 3.5 g/m² on a dry weight basis, followed by drying, whereby the upper layer was formed.

Thus, an intermediate layer comprising the lower layer as the main constituent layer and the upper layer as the protective layer was formed on the surface of the base paper sheet.

### Formation of image-receiving layer

### (a) Preparation of a coating composition:

100 parts of a polyester resin (trademark name: Vylon 200, produced by Toyobo Co., Ltd.), 0.5 parts of an amino-modified silicon (trademark name: KF-393, produced by The Shin-Etsu Chemical Co., Ltd.), and 0.5 parts of an epoxy-modified silicon (trademark name: X-22-343, produced by Shinetsu Chem. Ind. Co., Ltd.) were added to methyl ethyl ketone/toluene (ratio by weight of 1:1) while agitating with a mixer, to thereby obtain a coating composition for the image-receiving layer having a solid content of 15%.

### (b) Formation of the image-receiving layer

The coating composition obtained in the above was applied onto the surface of the upper layer of the intermediate layer in an amount to provide a thickness of 7 micrometers when dried by means of a wire bar, followed by drying. The resultant was subjected to supercalendering under the following conditions, to thereby form an image-receiving layer on the surface of the upper layer of the intermediate layer.

| Supercalendering conditions: | |
|---|---|
| linear pressure | 90 kg/cm |
| surface temperature of a chrominum-plated metal roll | 70°C |
| running paper speed | 5 m/minute |
| number of nips for running paper | 2 |

Thus, there was obtained an image-receiving sheet for thermal transfer printing.

### 2. A thermal transfer sheet was prepared in the following manner.

### (a) Preparation of an ink composition for the formation of a thermal transfer layer:

40 parts of a sublimable disperse dye (trademark name: Kayaset Blue 714, produced by Nippon Kayaku Co., Ltd.) and 60 parts by weight of polyvinyl butyral were added to methyl ethyl ketone/toluene (ratio by weight of 1:1) while agitating with a mixer to obtain an ink composition having a solid content of 10%.

### (b) Formation of a thermal transfer layer:

The ink composition obtained in the above was applied onto a 4.5 micrometer thick PET film, whose back side had been subjected to heat-resisting treatment, in an amount of 1 g/m² on a dry weight basis by means of a wire bar, followed by drying.

Thus, there was obtained a thermal transfer sheet.

### Evaluation of the image-receiving sheet for thermal transfer printing

The thermal transfer sheet obtained in the above was superposed on the image-receiving sheet for thermal transfer printing obtained in the above, followed by printing under conditions of an output power of 1 W/dot, a pulse width of 0.3 to 4.5 msec., and a dot density of 3 dots/mm for evaluation. The evaluated results are shown in Table 1.

### COMPARATIVE EXAMPLE 1

The procedures of Example 1 were repeated, except that the upper layer of the intermediate layer was not formed and after the formation of the lower layer, an image-receiving layer was formed directly on the lower layer, to thereby obtain an image-receiving sheet with a single-layered intermediate layer for thermal transfer printing.

As a result of examining the resultant image-receiving sheet, it was found that the solvent for the image-receiving layer infiltrated into the substrate, causing striking-through. It was also found that the thickness of the sheet prior to and after the formation of the image-receiving layer was reduced from 160 micrometers to 135 micrometers. This revealed that the intermediate layer was dissolved with the organic solvent for the image-receiving layer.

The sheet was evaluated in the same manner as in Example 1. The evaluated results are shown in Table 1.

### COMPARATIVE EXAMPLE 2

The procedures of Example 2 were repeated, except that the upper layer of the intermediate layer was not formed and after the formation of the lower layer, an image-receiving layer was formed directly on the lower layer, to thereby obtain an image-receiving sheet with a single-layered intermediate layer for thermal transfer printing.

As a result of examining the resultant image-receiving sheet, it was found that the sheet had fine wrinkles on the surface, revealing that the intermediate layer was swollen and dissolved with the organic solvent for the image-receiving layer.

The image-receiving sheet was evaluated in the same manner as in Example 1. The evaluated results are shown in Table 1.

Now, in Table 1, the evaluation methods for the respective tests are described below.

### 1. Resistance to organic solvent

The resistance was evaluated by visual observation and measurement of a sheet thickness.
- A: no problem
- E: no practical utility with a great number of defects

### 2. Anti-blocking properties

The intermediate layer and a black drawing paper were superposed and passed twice through a supercalender at a linear pressure of 50 kg/cm, after which the layer and the paper were separated from each other to observe the respective surfaces.
- A: little black fibers of the drawing paper transferred to the intermediate layer, and no practical problem
- E: the intermediate layer and the drawing paper bonded together

### 3. Optical density

The optical density of cyan color transferred onto the image-receiving layer was evaluated by the use of a reflection densitometer (Macbeth RD914).
- A: maximum value not less than 1.4
- B: maximum value of from 1.2 to 1.4
- C: maximum value of less than 1.2

### 4. Image quality

Evaluated through visual observation of missing transfer portion(s)
- AA: very excellent image quality with no missing transfer portion(s)
- A: little missing transfer portions observed with excellent image quality
- B: slight missing transfer portions observed with good image quality
- C: missing transfer portions observed but with no practical problem on image quality
- D: many missing transfer portions observed with poor image quality
- E: a great number of missing transfer portions observed with practically unacceptable image quality

**Table 1**

| | Example 1 | Example 2 |
|---|---|---|
| Base Sheet | wood free paper | same as in Example 1 |
| smoothness (%) | 13 | |
| water absorption degree (g/m ) | 10.4 | |

| Intermediate layer: | | |
|---|---|---|
| (i) main constituent of the lower layer (the main constituent layer) | (a) JSR-0696 (1) added ratio: 30 weight parts | (a) JSR-0696 (1) added ratio: 20 weight parts |
| | (b) Micro sphere F-30 (2) added ratio: 70 weight parts | (b) Ropaque OP-84J (4) added ratio: 80 weight parts |
| (ii) main constituent of the upper layer (the protective layer) | polyvinyl alcohol (3) | polyvinyl alcohol (3) |
| Resistance to solvents | A | A |
| Anti-blocking property | A | A |
| Optical density | A | A |
| Image quality | A | B |

| | Comparative Example 1 | Comparative Example 2 |
|---|---|---|
| Base Sheet | same as in Example 1 | same as in Example 1 |
| smoothness (%) | | |
| water absorption degree (g/m ) | | |

| Intermediate layer: | | |
|---|---|---|
| (i) main constituent of the lower layer (the main constituent layer) | same as in Example 1 | same as in Example 2 |
| (ii) main constituent of the upper layer (the protective layer) | none | none |
| Resistance to solvents | E | E |
| Anti-blocking property | A | A |
| Optical density | C | C |
| Image quality | E | E |
| (1) composition: styrene - 46wt.%, butadiene - 38wt.% gel content: 83wt.% (2) the trademark name of the product by Matsumoto Yushi-Seiyaku Co., Ltd. (3) product under the trademark name of PVA-110 by Kuraray Co., Ltd. (4) the trademark name of the product by Rohm & Haas Japan Kabushiki Kaisha | | |

## Claims

1. An image-receiving sheet for thermal transfer printing which comprises (a) an intermediate layer and (b) an image-receiving layer formed on a substrate in this order, characterized in that said intermediate layer (a) comprises (a-i) a lower layer and (a-ii) an upper layer formed on said lower layer (a-i), said image-receiving layer (b) being comprised primarily of a resin soluble in an organic solvent,
said lower layer (a-i) being comprised primarily of a resin insoluble in an organic solvent,
said resin being formed from a polymer latex satisfying the following requirements (1) and (2):
| | | |
|---|---|---|
| (1) | compositional constituents: | |
| | aliphatic conjugated diolefinic monomer | 20-70 wt.-% |
| | unsaturated acid monomer | 0.5-15 wt.-% |
| | other olefinic monomer | 15-79.5 wt.-% |
| (2) | gel content: | 85-100 wt.-% |
and containing hollow particles in an amount of not less than 50 wt.-% of the total solids in solid lower layer (a-i), the hollow particles having a size of 0.1-200 µm and being soluble in organic solvents, said upper layer (a-ii) being comprised of an organic-solvent resistant resin.

2. An image-receiving sheet for thermal transfer printing according to claim 1, wherein the lower layer of the intermediate layer further contains a binder resin.

3. An image-receiving sheet for thermal transfer printing according to claim 1, wherein the substrate is a paper sheet made primarily of pulp fibers.

4. An image-receiving sheet for thermal transfer printing according to claim 3, wherein the paper sheet has a smoothness of not less than 6% and a water absorption of from 1 to 30 g/m² when determined by the following procedures:
smoothness: a value measured by a specular reflection smoothness tester at a pressure of 20 kg/cm²; and
water absorption:: a 5 second value determined according to "a test method for water absorption of paper and paperboard (Cobb's method)" prescribed in JIS P-8140.

## Patentansprüche

1. Bildempfangsschicht für thermischen Übertragungsdruck, welche (a) eine Zwischenschicht und (b) eine Bildempfangsschicht, welche in dieser Reihenfolge auf einem Substrat gebildet wurden, umfaßt, dadurch **gekennzeichnet,** daß die Zwischenschicht (a) eine untere Schicht (a-i) und eine obere Schicht (a-ii), welche auf der unteren Schicht (a-i) gebildet wurde, umfaßt, daß die Bildempfangsschicht (b) hauptsächlich ein in einem organischen Lösungsmittel lösliches Harz umfaßt,
daß die untere Schicht (a-i) hauptsächlich ein in einem organischen Lösungsmittel unlösliches Harz umfaßt,
daß das Harz aus einem Polymerlatex gebildet ist, welches die folgenden Anforderungen (1) und (2) erfüllt:
| | | |
|---|---|---|
| (1) | Zusammensetzungsbestandteile: | |
| | aliphatisches konjugiertes diolefinisches Monomer | 20-70 Gew.-% |
| | ungesättigtes Säuremonomer | 0,5-15 Gew.-% |
| | weiteres olefinisches Monomer | 15-79,5 Gew.-% |
| (2) | Gelgehalt: | 85-100 Gew.-% |
und welches hohle Teilchen in einer Menge von nicht weniger als 50 Gew.-% der gesamten Feststoffe in der festen unteren Schicht (a-i) enthält, wobei die hohlen Teilchen eine Größe von 0,1-200 µm besitzen und in organischen Lösungsmitteln löslich sind, wobei die obere Schicht (a-ii) ein gegenüber organischen Lösungsmitteln beständiges Harz umfaßt.

2. Bildempfangsschicht für thermischen Übertragungdruck nach Anspruch 1, dadurch **gekennzeichnet,** daß die untere Schicht der Zwischenschicht ferner ein Binderharz enthält.

3. Bildempfangsschicht für thermischen Übertragungsdruck nach Anspruch 1, dadurch **gekennzeichnet,** daß das Substrat ein Blatt Papier ist, welches hauptsächlich aus Zellstoffasern hergestellt wurde.

4. Bildempfangsschicht für thermischen Übertragungsdruck nach Anspruch 3, dadurch **gekennzeichnet,** daß das Blatt Papier eine Glattheit von nicht weniger als 6% und eine Wasserabsorption von 1 bis 30 g/m² besitzt, wenn mittels der folgenden Verfahren die Bestimmungen durchgeführt werden:
Glattheit: Wert, gemessen mit einem Rückspiegelungs-Glattheitsprüfer bei einem Druck von 20 kg/cm²; und
Wasserabsorption: 5-Sekunden-Wert, bestimmt gemäß "einem Testverfahren für Wasserabsorption von Papier und Pappe (Verfahren nach Cobb)", beschrieben in JIS P-8140.

## Revendications

1. Feuille réceptrice d'image pour l'impression par transfert thermique, qui comprend (a) une couche intermédiaire et (b) une couche de réception d'image formées dans cet ordre sur un substrat, caractérisée en ce que cette couche intermédiaire (a) comprend (a-i) une couche inférieure et (a-ii) une couche supérieure formée sur cette couche inférieure (a-i), cette couche de réception d'image (b) étant principalement composée d'une résine soluble dans un solvant organique,
cette couche inférieure (a-i) étant principalement composée d'une résine insoluble dans un solvant organique,
cette résine étant formée à partir d'un latex de polymère satisfaisant aux conditions requises (1) et (2) suivantes :
| | | |
|---|---|---|
| (1) | constituants de la composition : | |
| | monomère dioléfinique conjugué aliphatique | 20 à 70% en poids |
| | monomère acide insaturé | 0,5 à 15% en poids |
| | autre monomère oléfinique | 15 à 79,5% en poids |
| (2) | teneur en gel : | 85 à 100% en poids |
et contenant des particules creuses en une quantité d'au moins 50% en poids des solides totaux dans la couche inférieure solide (a-i), les particules creuses ayant une dimension de 0,1 à 200 µm et étant solubles dans des solvants organiques, cette couche supérieure (a-ii) étant composée d'une résine résistant aux solvants organiques.

2. Feuille réceptrice d'image pour l'impression par transfert thermique selon la revendication 1, dans laquelle la couche inférieure de la couche intermédiaire contient de plus une résine de liaison.

3. Feuille réceptrice d'image pour l'impression par transfert thermique selon la revendication 1, dans laquelle le substrat est une feuille de papier faite principalement de fibres de pulpe.

4. Feuille réceptrice d'image pour l'impression par transfert thermique selon la revendication 3, dans laquelle la feuille de papier a une égalité de surface d'au moins 6% et une absorption d'eau de 1 à 30 g/m² lorsqu'elles sont déterminées selon les procédures suivantes :
égalité de surface : valeur mesurée par un appareil de test de l'égalité de surface par réflexion spéculaire sous une pression de 20 kg/cm²; et
absorption d'eau : une valeur pour 5 secondes déterminée selon "une procédure d'essai pour l'absorption d'eau par le papier et le carton (procédé de Cobb)" prescrite dans JIS P-8140.
